

## UNITED STATES PATENT OFFICE.

HARRY A. SCHWARTZ, OF CLEVELAND HEIGHTS, OHIO, ASSIGNOR TO NATIONAL MALLEABLE AND STEEL CASTINGS COMPANY, OF CLEVELAND, OHIO, A CORPORATION OF OHIO.

## MANUFACTURE OF MALLEABLE CAST IRON.

No Drawing.

Application filed October 22, 1926. Serial No. 143,511.

My invention relates to the manufacture of malleable cast iron, and particularly to the overcoming of graphitization difficulties normally met within the annealing operation in such manufacture.

It is well known that elements such as sulphur, selenium and tellurium, which form readily non-metallic compounds with iron, are a detriment to annealing. This is usually attributed (as when sulphur is present) to the formation of films or networks of sulphides about the iron and iron-carbon crystals which hinder the migration of carbon during annealing. In practice this difficulty is usually overcome by adding sufficient manganese, which readily combines with the sulphur to form globules of manganese sulphide instead of iron sulphide films. If, however, too great an excess of manganese is added, this also interferes with annealing, and where the percent of sulphur is variable and not known in advance there is danger of having a harmful excess of manganese when the sulphur is less than is anticipated.

I have found, however, that if, instead of manganese, a rare earth element such as cerium is added, just before pouring the molten metal, in a quantity in the ratio of its atomic weight to that of the sulphur and other similar elements present in the iron but preferably more than sufficient to combine with all the sulphur and similar elements, such an element combines with the sulphur content more easily than such elements as manganese or tin, and, as the resulting sulphide forms as globules rather than a network it is innocuous so far as its effect on graphitization is concerned, and as its excess over that necessary to form the sulphide is not harmful in annealing it is not a matter of importance, except for the sake of economy, whether the excess is large or not. Normally the cerium addition is approximately .25% to .50% and is added preferably in the form of Misch metal just before the metal is tapped, or in the ladle. As substantially all of the sulphur readily combines with the cerium, the manganese is left free to alloy with the metal itself. Hence, by the use of cerium the effects of sulphur, selenium and tellurium on graphitization may be completely controlled without the necessity of carefully regulating the controlling factor, as is the case with manganese.

A typical iron used for making malleable iron contains carbon 2.50%, silicon .80%, manganese .26%, sulphur .07%, phosphorus .18%. If the sulphur is to be counteracted by cerium it is not necessary to have such high manganese, and the amount of manganese would be controlled to avoid interference with annealing by that element.

I have found also that so far as tin is concerned, as the sulphur combines with the cerium more readily than it does with tin, the harmful effect of the tin sulphide, which is more pronounced than iron sulphide, is prevented, and the tin, since all of the sulphur has been taken up by the cerium as cerium sulphide, will, like the manganese in small excess, combine with the iron in such a way as not to impair the qualities of the iron.

I have observed that where iron sulphide forms in the making of malleable iron, as its melting point is lower than that of the bulk of the mass, it solidifies after the iron and iron-carbon compounds and thus has the opportunity of forming a network or series of films around the already formed iron and iron-carbon crystals which seriously retards graphitization during annealing, as such network or series of films interferes with the separation of the carbon from the mass in the form of temper carbon.

I have also observed that normally a rare earth metal such as cerium will combine with the sulphur to form a compound the melting point of which is above that of the mass as a whole, and when the mass cools this compound will freeze out of the mass as globules or included grains which will not hinder graphitization, as where iron sulphide forms. In other words, a rare earth metal, as it has a greater affinity for sulphur than does iron, and as its sulphide has a higher melting point than the bulk of the molten mass, solidifies while the rest of the mass is liquid and is thus free to form the globules or included grains which in the subsequent annealing operation do not hinder the separation of the carbon from the iron-carbon compounds.

It will thus be seen that by the use of cerium, which does not have to be regulated in amount as does manganese because an excess has no harmful effect, I have provided an element which very effectively renders in-

nocuous such metalloids as sulphur, selenium and tellurium.

The employment of my invention is, however, not limited to the addition of cerium, but any other element of the cerium group, such as lanthanum, neodymium, praseodymium, erbium or europium, which is or may be commercially available, may be employed in amounts substantially proportional to the ratio of their respective atomic weights to that of cerium.

It will therefore be seen that to achieve the beneficial results of my invention the added element must have a greater affinity for the harmful metalloid (as sulphur) than has the other element (as iron) of the original compound; that the melting point of its compound with the metalloid should be higher than that of the bulk of the mass; and that it is desirable that its presence in excess over that required to combine with the metalloid be not harmful to graphitization.

The terms and expressions which I have employed are used as terms of description and not of limitation, and I have no intention, in the use of such terms and expressions, of excluding any equivalents of the features shown and described, or portions thereof, but recognize that various modifications are possible within the scope of the invention claimed.

What I claim is:

1. That improvement in the art of making malleable iron castings which comprises melting the iron, adding to the molten iron a rare earth element having a greater affinity for a metalloid contained in the molten iron, such as sulphur, than it has for the iron, casting the metal, whereby as the mass cools the element combined with the metalloid freezes out of the mass in the form of included globules at a higher temperature than the freezing point of the bulk of the mass, and in which the presence of the element in excess of the amount required to combine with the metalloid is not harmful to graphitization.

2. That improvement in the art of making malleable iron castings which comprises melting the iron, adding to the molten iron an element of the cerium group having a greater affinity for a metalloid contained in the molten iron, such as sulphur, than it has

for the iron, casting the metal, whereby as the mass cools the element combined with the metalloid freezes out of the mass in the form of included globules at a higher temperature than the freezing point of the bulk of the mass, and then the mass freezes at a lower temperature, whereby the combined carbon is free to separate out of the mass during the subsequent annealing operation, the presence of the element in excess of the amount required to combine with the metalloid not being harmful to graphitization.

3. That improvement in the art of making malleable iron castings which comprises melting the iron, adding to the molten iron an element of the cerium group, casting the metal, whereby as the mass cools the element combined with a metalloid present in the iron freezes out of the same in the form of included globules at a higher temperature than the freezing point of the bulk of the mass and in which the presence of the element in excess of the amount required to combine with the metalloid is not harmful to graphitization.

4. That improvement in the art of making malleable iron castings which comprises melting the iron containing metalloids such as sulphur, adding cerium to the molten iron and casting the metal, whereby as the mass cools the cerium combined with the sulphur first freeze out of the mass as cerium sulphide in the form of included globules and then the mass as a whole freezes, thereby rendering the combined carbon in the mass free to separate out as temper carbon in the subsequent annealing operation.

5. That improvement in the art of making malleable iron castings which comprises melting the iron containing elements having an affinity for each other such as tin and sulphur, which normally form non-metallic compounds in the iron, adding a rare earth element having a greater affinity for the sulphur than it has for the tin or the iron, and casting the metal, whereby as the mass cools the added element combined with the sulphur freezes out of the mass and the formation of sulphide of tin is thus avoided.

HARRY A. SCHWARTZ.